

April 21, 1942.

T. R. JONES

2,280,706

PROCESS FOR PURIFYING METALS

Filed March 20, 1941

Fig. 1.



Fig. 2.

INVENTOR  
THOMAS R. JONES  
BY  
*Ward, Crosby & Neal*  
ATTORNEYS

## UNITED STATES PATENT OFFICE

2,280,706

## PROCESS FOR PURIFYING METALS

Thomas R. Jones, Woodbridge, N. J., assignor to  
 The American Metal Company, Limited, New  
 York, N. Y., a corporation of New York

Application March 20, 1941, Serial No. 384,260

12 Claims.

(Cl. 75—85)

My invention relates to a process of removing lead from tin and is especially useful in removing small amounts of lead from otherwise pure tin. My invention has further reference to apparatus for performing the described process and such other metal-separating processes as may be suitable or desirable.

It is well known that in removing small amounts of lead from tin by chlorination at low temperatures the resultant dross is low in lead chloride and high in stannous chloride. It is also known that, if the operation of removing lead from tin by chlorination is carried on at high temperatures, both lead and stannous chlorides may be volatilized and must then be collected in condensing systems wherein a separation of the products may be attempted. It is evident that this type of process requires elaborate apparatus and, due to the corrosiveness of the products, presents a serious and difficult problem in construction and operation. There have been many other methods and apparatus proposed for the separation of lead and tin by means of chlorine and chlorides, but none have had the simplicity, practicability and novelty of my invention.

I have devised a process and apparatus in which a bath of molten tin containing some lead may be reduced in lead content to less than 0.05 percent. The lead is recovered as a retort residue by distilling  $\text{SnCl}_2$  away from a  $\text{SnCl}_2\text{-PbCl}_2$  mixture and returning the lead-free  $\text{SnCl}_2$  to a tin de-leading kettle.

The removal of lead from tin by means of chlorine depends upon the greater affinity of chlorine for lead than for tin. If a lead-tin alloy is treated with a given amount of chlorine, a  $\text{PbCl}_2\text{-SnCl}_2$  dross forms on the metal, in which the lead-tin ratio eventually comes to a definite figure depending on the final lead-tin ratio of the alloy upon which the dross rests. The reaction  $\text{Pb} + \text{SnCl}_2 \rightarrow \text{PbCl}_2 + \text{Sn}$  is reversible. To force it to go in either direction, it is necessary to remove one of the products of the reaction in order to prevent attainment of equilibrium between alloy and dross composition.

My invention is based on the principle that if  $\text{SnCl}_2$  is continually added to the lead-tin, lead chloride, stannous-chloride system shown above, the reaction will go from left to right, and that if the  $\text{PbCl}_2$  is continuously removed from the system, then eventually substantially all of the lead will be removed from the tin.

In order to do this, I remove  $\text{PbCl}_2\text{-SnCl}_2$  55 adjacent the retort 10.

dross from the metal bath continuously and place it in a retort where the dross is raised in temperature in order to distill off the  $\text{SnCl}_2$  which is returned to the metal bath where it reacts with the lead of the metal bath to form  $\text{PbCl}_2$  and metallic tin according to the above mentioned equation, thereby repressing the formation of more  $\text{SnCl}_2$  and accelerating the formation of  $\text{PbCl}_2$ . By this procedure, the  $\text{PbCl}_2$  10 continuously accumulates in the retort, whereas the  $\text{SnCl}_2$  is continually circulating and being drawn off to the retort with some lead. In this way, practically all the lead may be removed from the tin.

15 On the accompanying drawing:

Figure 1 is a vertical sectional view, partly in elevation, showing one form of apparatus suitable for practicing the invention; and

Fig. 2 is a plan view, partly in section, of the 20 apparatus shown in Fig. 1.

As shown on the drawing, 1 represents a de-leading kettle which is mounted on a suitable support 2. The kettle 1 is closed by a cover plate 3 suitably anchored in closing position. 25 An electrical motor 4 carried by a suitable support 5 operates a depending, vertical shaft 6 which extends downwardly thru the cover plate 3 and, at its lower end, carries an agitator 7.

Suitably secured to the interior surface of the 30 kettle 1 is an angular member 8 which forms a chamber or dross trap open at its upper and lower sides. The kettle 1 is provided with an opening 1a which places the dross trap in communication with an inclined conduit 9 adapted 35 to discharge into a suitably supported retort 10 closed by a cover plate 11. Adjacent its upper end, the retort 10 has a second inclined conduit 12 communicating therewith, said conduit 12 extending toward and opening into a vertical pipe 13 adapted to discharge into the kettle 1 40 thru an opening 3a provided in the cover plate 3, the pipe 13 being closed by a detachable plug 14.

In accordance with the invention, the cover 45 plate 3 may carry a funnel 15 adapted to be closed or sealed by a slide plate 16. In addition, said cover plate 3 may carry a pipe 17 adapted to be closed by a valve 18. As indicated, the funnel 15 and the pipe 17 communicate with the kettle 1 thru openings provided, respectively, therefor in the cover plate 3.

Further, as shown, a suitable heating device 19 should be associated with the kettle 1 and, similarly, a heating device 20 should be disposed 50 adjacent the retort 10.

After a suitable quantity of melted lead-containing tin has been pumped or otherwise suitably passed into the kettle 1, the operation proceeds in the following manner. Initially, it is necessary to provide a cover or upper layer of  $\text{SnCl}_2$  on the melted lead-containing tin and this may be accomplished in any one of a variety of ways. Thus, a  $\text{SnCl}_2$  dross may be introduced into the kettle 1 by passage thereof thru the funnel 15 after the slide plate 16 has been opened, the latter being closed after the desired amount of  $\text{SnCl}_2$  dross has been passed into said kettle 1. Alternatively, in order to chlorinate some of the tin, chlorine gas may be passed into the kettle 1 by way of the valve-controlled pipe 17. In lieu of the foregoing,  $\text{SnCl}_2$  vapor may be passed into the kettle 1 from the retort 10 which, as hereinafter described, constitutes a source of supply of such vapor.

After completion of the foregoing, the heating device 19 is operated to maintain the temperature of the metal bath in the kettle 1 in a range varying between 470 degrees F. and 600 degrees F. At this time, the motor 4 is energized to rotate the agitator 7 at suitable speed whereby the  $\text{SnCl}_2$  reacts with the lead to form a dross layer *d* of  $\text{PbCl}_2$  and  $\text{SnCl}_2$  on the tin metal bath *b*. During this operation, the dross layer collects in the dross trap formed by the member 8 from which the collected dross flows thru the pipe 9 and passes into the retort 10, this operation proceeding in a continuous manner as will be understood.

While the foregoing operation proceeds, the burner 20 should be operated to maintain the material in the retort 10 at a temperature ranging between 1200 degrees F. and 1300 degrees F. This causes the  $\text{SnCl}_2$  to distill away from the lead chloride and return, by way of the conduit 12, to the kettle 1 and again enter into reaction with the metallic lead therein so as to form additional lead chloride which, in turn, as a dross passes to the retort 10 to continue the process. In this connection, it will be understood that the vapor pressure in the retort 10 becomes sufficiently high to pass  $\text{SnCl}_2$  vapor from said retort 10 to the kettle 1 by way of the conduit 12, condensing in said conduit or kettle.

Eventually, in the manner described, substantially all of the lead is removed from the tin in the kettle 1, the lead thus removed remaining in the retort 10 as will be understood. As the process nears its conclusion, the temperature of the material in said retort 10 may be increased as high as 1500 degrees F., this high temperature being utilized in order to drive off as much  $\text{SnCl}_2$  from the retort 10 as possible while not bringing the temperature sufficiently high to vaporize lead chloride. This assures the highest possible lead content of the lead residue remaining in the retort 10. This lead residue is removed from the retort 10 from time to time depending on the amount of lead present in the original tin charged into the kettle 1. The stannous chloride is smelted to recover the tin.

I have found that an ordinary iron retort 10, when used in performing the described process, does not last very long due to the corrosive action of  $\text{PbCl}_2$  and  $\text{SnCl}_2$ . Special alloys or a metal such as copper or the like are necessary in commercial practice. I have found that "Hastelloy B" withstands the corrosive action very well.

While the invention has been described in de-

tail according to the preferred manner of carrying out the process, it will be obvious to those skilled in the art after understanding the invention, that changes and modifications may be made therein without departing from the spirit or scope of the invention, and it is intended in the appended claims to cover all such changes and modifications.

What is claimed as new and desired to be secured by Letters Patent, is:

1. The process of removing lead as an impurity from tin, which comprises forming a dross of stannous chloride and lead chloride on a mass of molten tin containing the lead impurity, passing the dross away from the molten tin and separating the stannous chloride from the lead chloride.

15 2. The process of removing lead as an impurity from tin, which comprises forming a dross of stannous chloride and lead chloride on a mass of molten tin containing the lead impurity, passing the dross to a retort, maintaining the retort temperature sufficiently high to cause the stannous chloride to distill from the lead chloride, and returning the stannous chloride to the zone occupied by said mass of molten tin.

20 3. The process of removing lead as an impurity from tin, which comprises forming a dross of stannous chloride and lead chloride on a mass of molten tin containing the lead impurity, trapping the dross and passing the same to a retort under the action of gravity, maintaining the retort temperature sufficiently high to cause the stannous chloride to distill from the lead chloride, and, responsive to the pressure existing in said retort, returning the stannous chloride to the zone occupied by said mass of molten tin.

25 4. The process of removing lead as an impurity from tin, which comprises melting the tin having the lead impurity therein, producing a layer of stannous chloride on the surface of the molten metal, agitating the molten metal to cause the stannous chloride to react with the lead and thereby produce a dross of stannous chloride and lead chloride, elevating the temperature of the dross after removal thereof from the melting zone to distill the stannous chloride from the lead chloride, and returning the stannous chloride to the melting zone.

30 5. The process of removing lead as an impurity from tin, which comprises melting the tin having the lead impurity therein, producing a layer of stannous chloride on the surface of the molten metal, agitating the molten metal to cause the stannous chloride to react with the lead and thereby produce a dross of stannous chloride and lead chloride, passing the dross to a zone wherein the stannous chloride is separated from the lead chloride, and returning the stannous chloride to the melting zone.

35 6. The process of removing lead as an impurity from tin, which comprises melting the tin having the lead impurity therein, producing a layer of stannous chloride on the surface of the molten metal, agitating the molten metal to cause the stannous chloride to react with the lead and thereby produce a dross of stannous chloride and lead chloride, trapping the dross and passing the same to a retort under the action of gravity, maintaining the retort temperature sufficiently high to cause the stannous chloride to distill from the lead chloride, and returning the stannous chloride to the melting zone.

40 7. The process of removing lead as an impurity from tin, which comprises melting the tin having the lead impurity therein, producing a layer

of stannous chloride on the surface of the molten metal, agitating the molten metal, while maintaining the temperature thereof between 470 degrees F. and 600 degrees F., to cause the stannous chloride to react with the lead and thereby produce a dross of stannous chloride and lead chloride, passing the dross to a retort, maintaining the retort temperature between 1200 degrees F. and 1300 degrees F. to cause the stannous chloride to distill from the lead chloride, and returning the stannous chloride to the melting zone.

8. The process of removing lead as an impurity from tin, which comprises melting the tin having the lead impurity therein, producing a layer of stannous chloride on the surface of the molten metal, agitating the molten metal, while maintaining the temperature thereof between 470 degrees F. and 600 degrees F., to cause the stannous chloride to react with the lead and thereby produce a dross of stannous chloride and lead chloride, passing the dross to a retort, maintaining the retort temperature between 1200 degrees F. and 1300 degrees F. to cause the stannous chloride to distill from the lead chloride, and, when the tin in the melting zone becomes substantially free from lead, elevating the retort temperature to 1500 degrees F. approximately.

9. In the art of removing lead as an impurity from tin, the steps which consist in continuously passing a dross of stannous chloride and lead chloride from a kettle to a retort, distilling the stannous chloride from the lead chloride in the retort, and continuously passing the stannous chloride vapor from the retort to the kettle.

10. In the art of removing lead as an impurity from tin, the steps which consist in continuously passing a dross of stannous chloride and lead chloride to a retort from a kettle containing the tin and the lead impurity in molten condition, distilling the stannous chloride from the lead

chloride in the retort, continuously passing the stannous chloride vapor from the retort to the kettle, and agitating the molten metal in the kettle to cause the stannous chloride to react with the lead and thereby produce a further dross supply of stannous chloride and lead chloride.

11. In the art of removing lead as an impurity from tin, the steps which consist in continuously passing a dross of stannous chloride and lead chloride to a retort from a kettle containing the tin and the lead impurity in molten condition, maintaining the retort temperature between 1200 degrees F. and 1300 degrees F. to cause the stannous chloride to distill from the lead chloride, continuously passing the stannous chloride vapor from the retort to the kettle, and agitating the molten metal in the kettle, while maintaining the temperature thereof approximately between 470 degrees F. and 600 degrees F., to cause the stannous chloride to react with the lead and thereby produce a further dross supply of stannous chloride and lead chloride.

12. In the art of removing lead as an impurity from tin, the steps which consist in continuously passing a dross of stannous chloride and lead chloride to a retort from a kettle containing the tin and the lead impurity in molten condition, maintaining the retort temperature initially between 1200 degrees F. and 1300 degrees F. and subsequently at 1500 degrees F. approximately to cause the stannous chloride to distill from the lead chloride, continuously passing the stannous chloride vapor from the retort to the kettle, and agitating the molten metal in the kettle, while maintaining the temperature thereof approximately between 470 degrees F. and 600 degrees F., to cause the stannous chloride to react with the lead and thereby produce a further dross supply of stannous chloride and lead chloride.

THOMAS R. JONES.